# EUROPEAN PATENT SPECIFICATION

(11) **EP 3 279 292 B1**
(45) Date of publication and mention of the grant of the patent: **01.05.2024**
(21) Application number: 16772852.6
(22) Date of filing: 29.03.2016
(51) Int. Cl.: C10M 141/12, C10M 101/02, C10M 107/02, C10M 129/68, C10M 129/76, C10M 133/04, C10M 135/18, C10M 137/10, C10M 139/00, C10M 145/14, C10N 10/04, C10N 10/12, C10N 30/00, C10N 30/06, C10N 40/25, C10M 141/08

(54) **LUBRICANT OIL COMPOSITION AND INTERNAL-COMBUSTION-ENGINE FRICTION REDUCTION METHOD**
SCHMIERÖLZUSAMMENSETZUNG UND REIBUNGSVERRINGERUNGSVERFAHREN FÜR BRENNKRAFTMASCHINE
COMPOSITION D'HUILE LUBRIFIANTE ET PROCÉDÉ DE RÉDUCTION DE FROTTEMENT DE MOTEUR À COMBUSTION INTERNE

(30) Priority: 31.03.2015 JP 2015074366
(43) Date of publication of application: 07.02.2018
(73) Proprietor: Idemitsu Kosan Co.,Ltd., Chiyoda-ku Tokyo 100-8321 (JP)
(72) Inventor: NAKAYA, Ikuko, Ichihara-shi Chiba 299-0107 (JP); TAMURA, Kazushi, Ichihara-shi Chiba 299-0107 (JP)
(74) Representative: Hoffmann Eitle
(86) International application number: PCT/JP2016/060168
(87) International publication number: WO 2016/158971

(56) References cited:
- EP-A1- 2 080 798
- EP-A1- 2 133 406
- WO-A1-2005/014763
- WO-A1-2010/032781
- WO-A1-2014/021350
- WO-A1-2014/021350
- WO-A1-2015/022976
- WO-A2-2012/071185
- JP-A- H07 150 173
- JP-A- 2003 073 685
- JP-A- 2003 221 588
- JP-A- 2004 277 712
- JP-A- 2006 182 986
- JP-A- 2008 106 199
- JP-A- 2009 292 998
- JP-A- 2010 100 707
- JP-A- 2011 195 774
- JP-A- 2015 140 354

## Description

### Technical Field

The present invention relates to a lubricating oil composition and a method for reducing friction of an internal combustion engine.

### Background Art

In recent years, following the strengthening of environmental regulations, high fuel consumption reducing properties have been required for engine oils. For this reason, efforts have been made regarding blending a molybdenum compound such as molybdenum dithiocarbamate (MoDTC) into a lubricating oil composition, thereby reducing a metal-to-metal friction coefficient.

The molybdenum compound such as MoDTC exhibits a friction-reducing effect in a relatively high temperature region of 80°C or higher. Examples of the lubricating oil composition having a molybdenum compound blended therein include those disclosed in PTL 1.

Meanwhile, ashless friction modifiers such as an ester-based friction modifier and an amine-based friction modifier are also used so as to reduce friction (for example, PTL 2).

These ashless friction modifiers have excellent friction-reducing effects in a relatively low temperature region of lower than 80°C.

Taking into consideration the friction-reducing characteristics of a molybdenum compound in a high-temperature region and the friction-reducing characteristics of an ashless friction modifier in a low-temperature region, it can be expected that a friction-reducing effect is exhibited in a wide temperature region by using a molybdenum compound in combination with an ashless friction modifier. EP 2 080 798 A1 relates to a lubricating oil for internal combustion engines comprising a base oil for a lubricating oil, sulfated oxymolybdenum dithiocarbamate, an acid amide compound a fatty acid partial ester compound and/or an aliphatic amide compound, and a benzotriazole derivative. WO 2012/071185 A2 relates to a lubricating oil composition comprising an oil of lubricating viscosity and from 0.25 to 5 weight percent based upon the total mass of the lubricating oil composition of a friction modifier composition comprising an amino alcohol reaction product and an ester of glycerol and a C₁₂-C₂₂ carboxylic acid containing 0 to 3 double bonds.

### Citation List

### Patent Literature

PTL 1: JP 2015-010177 A
PTL 2: WO 2011/062282 A

### Summary of Invention

### Technical Problem

However, in a case of using a molybdenum compound in combination with an ashless friction modifier, there was involved such a problem that the ashless friction modifier inhibits a friction-reducing effect of the molybdenum compound, and consequently, impairs fuel consumption reducing properties.

It is an object of the present invention to provide a lubricating oil composition which exhibits an excellent friction-reducing effect and excellent fuel consumption reducing properties.

### Solution to Problem

In order to solve the aforementioned problem, an embodiment of the present invention provides a lubricating oil composition including a lubricating base oil (A), a molybdenum compound (B), an ashless friction modifier (C), and a borated succinimide (D),
wherein the lubricating oil composition includes a binuclear organic molybdenum compound represented by the following general formula (I) as the molybdenum compound (B), with the content of the binuclear organic molybdenum compound as converted into molybdenum atoms being 0.030 mass% or more and 0.140 mass% or less based on the total amount of the lubricating oil composition; and
an ester-based ashless friction modifier (C1) and an amine-based ashless friction modifier (C2) as the ashless friction modifier (C), with the total content of the ester-based ashless friction modifier (C1) and the amine-based ashless friction modifier (C2) being more than 0.1 mass% and 1.8 mass% or less based on the total amount of the lubricating oil composition:
in the general formula (I), R¹ to R⁴ each represents a hydrocarbon group having 4 to 22 carbon atoms, R¹ to R⁴ may be the same as or different from each other, and X¹ to X⁴ each represents a sulfur atom or an oxygen atom,
wherein the amine-based ashless friction modifier (C2) is an aliphatic amine-based compound having one or more hydroxyl groups in a molecule thereof,
wherein the mass ratio between the content of the amine-based ashless friction modifier (C2) and the content of the ester-based ashless friction modifier (C1) [the content of the amine-based ashless friction modifier (C2)/the content of the ester-based ashless friction modifier (C1)] is 0.15 or more and 0.80 or less.

### Advantageous Effect of Invention

Since the lubricating oil composition of the present invention makes it possible to use the molybdenum compound in combination with an ashless friction modifier without inhibiting the friction-reducing effect of a molybdenum compound, the lubricating oil composition exhibits an excellent friction-reducing effect and can enhance fuel consumption reducing properties.

### Description of Embodiments

Hereinafter, an embodiment of the present invention will be described. [Lubricating Oil Composition]

The lubricating oil composition of the present embodiment is a lubricating oil composition including a lubricating base oil (A), a molybdenum compound (B), an ashless friction modifier (C), and a borated succinimide (D),
wherein the lubricating oil composition includes a binuclear organic molybdenum compound represented by the following general formula (I) as the molybdenum compound (B), with the content of the binuclear organic molybdenum compound as converted into molybdenum atoms being 0.030 mass% or more and 0.140 mass% or less based on the total amount of the lubricating oil composition; and
an ester-based ashless friction modifier (C1) and/or an amine-based ashless friction modifier (C2) as the ashless friction modifier (C), with the total content of the ester-based ashless friction modifier (C1) and the amine-based ashless friction modifier (C2) being more than 0.1 mass% and 1.8 mass% or less based on the total amount of the lubricating oil composition:
in the general formula (I), R¹ to R⁴ each represents a hydrocarbon group having 4 to 22 carbon atoms, R¹ to R⁴ may be the same as or different from each other, and X¹ to X⁴ each represents a sulfur atom or an oxygen atom,
wherein the amine-based ashless friction modifier (C2) is an aliphatic amine-based compound having one or more hydroxyl groups in a molecule thereof,
wherein the mass ratio between the content of the amine-based ashless friction modifier (C2) and the content of the ester-based ashless friction modifier (C1) [the content of the amine-based ashless friction modifier (C2)/the content of the ester-based ashless friction modifier (C1)] is 0.15 or more and 0.80 or less.

### <(A) Lubricating Base Oil>

The lubricating oil composition of the present embodiment includes a lubricating base oil (A). Examples of the lubricating base oil as the component (A) include a mineral oil and/or a synthetic oil.

Examples of the mineral oil include a paraffin-based mineral oil, an intermediate-based mineral oil, and a naphthene-based mineral oil, obtained by a usual refining method such as solvent refining and hydrogenation refining; and wax-isomerized oils produced by isomerizing a wax such as a wax (a gas-to-liquid wax) produced by a Fischer-Tropsch process or the like, and a mineral oil-based wax.

Examples of the synthetic oil include a hydrocarbon-based synthetic oil and an ether-based synthetic oil. Examples of the hydrocarbon-based synthetic oil include an α-olefin oligomer such as polybutene, polyisobutylene, a 1-octene oligomer, a 1-decene oligomer, and an ethylene-propylene copolymer, or a hydride thereof; an alkylbenzene; and an alkylnaphthalene. Examples of the ether-based synthetic oil include polyoxyalkylene glycol and polyphenyl ether.

Although the lubricating base oil (A) may be of a single system using one of the aforementioned mineral oils and synthetic oils, it may also be of a mixed system, for example, a mixture of two or more mineral oils, a mixture of two or more synthetic oils, or a mixture of each one or each two or more of mineral oils and synthetic oils.

In particular, it is preferable to use one or more selected from mineral oils or synthetic oils classified into Group 3 and Group 4 in the base oil classification of the American Petroleum Institute as the lubricating base oil (A).

The content of the lubricating base oil (A) is preferably 60 mass% or more, more preferably 65 mass% or more and 95 mass% or less, and still more preferably 70 mass% or more and 85 mass% or less, based on the total amount of the lubricating oil composition.

### <Molybdenum Compound (B)>

The lubricating oil composition of the present embodiment includes a molybdenum compound (B). Further, the lubricating oil composition of the present embodiment includes a binuclear organic molybdenum compound represented by the following general formula (I) as the molybdenum compound of the component (B), and the content of the binuclear organic molybdenum compound as converted into molybdenum atoms is 0.030 mass% or more and 0.140 mass% or less based on the total amount of the lubricating oil composition.

In the general formula (I), R¹ to R⁴ each represents a hydrocarbon group having 4 to 22 carbon atoms, and R¹ to R⁴ may be the same as or different from each other. When the number of carbon atoms is 3 or less, the oil solubility becomes poor, whereas when the number of carbon atoms is 23 or more, the melting point becomes high, the handling becomes deteriorated, and the friction-reducing ability becomes low. From the viewpoints, the number of carbon atoms is preferably 4 to 18, and more preferably 8 to 13.

Examples of the hydrocarbon group of R¹ to R⁴ include an alkyl group, an alkenyl group, an alkylaryl group, a cycloalkyl group, and a cycloalkenyl group. A branched or linear alkyl group or alkenyl group is preferable, and a branched or linear alkyl group is more preferable. Examples of the branched or linear alkyl group include an n-octyl group, a 2-ethylhexyl group, an isononyl group, an n-decyl group, an isodecyl group, a dodecyl group, a tridecyl group, and an isotridecyl group.

Furthermore, from the viewpoints of solubility in the base oil, storage stability, and friction-reducing ability, in the binuclear organic molybdenum compound represented by the general formula (I), it is preferable that R¹ and R² are the same alkyl group, R³ and R⁴ are the same alkyl group, and the alkyl groups of R¹ and R² and the alkyl groups of R³ and R⁴ are different from each other.

Moreover, in the general formula (I), X¹ to X⁴ each represents a sulfur atom or an oxygen atom, and X¹ to X⁴ may be the same as or different from each other. The ratio of the sulfur atoms to the oxygen atoms is preferably 1/3 to 3/1, and more preferably 1.5/2.5 to 3/1 as converted into sulfur atoms/oxygen atoms. When the ratio falls within the range, good performance is obtained in view of corrosion resistance and solubility in a lubricating base oil. In addition, all of X¹ to X⁴ may also be a sulfur atom or an oxygen atom.

In the lubricating oil composition of the present embodiment, the content of the binuclear organic molybdenum compound as converted into molybdenum atoms needs to be 0.030 mass% or more and 0.140 mass% or less based on the total amount of the lubricating oil composition.

In a case where the content of the binuclear organic molybdenum compound as converted into molybdenum atoms is less than 0.030 mass%, the friction-reducing effect in a high-temperature region cannot be enhanced, and thus, fuel consumption reducing properties cannot be satisfied. Further, in a case where the content of the binuclear organic molybdenum compound as converted into molybdenum atoms is more than 0.140 mass%, cleanness is deteriorated.

The content of the binuclear organic molybdenum compound as converted into molybdenum atoms is preferably 0.050 to 0.120 mass%, and more preferably 0.060 to 0.100 mass%, based on the total amount of the lubricating oil composition.

In addition, the lubricating oil composition of the present embodiment may further contain a mononuclear organic molybdenum compound and/or a trinuclear organic molybdenum compound as the molybdenum compound.

### <Ashless Friction Modifier (C)>

The lubricating oil composition of the present embodiment includes an ashless friction modifier (C). Further, the lubricating oil composition of the present embodiment includes an ester-based ashless friction modifier (C1) and an amine-based ashless friction modifier (C2) as the ashless friction modifier of the component (C), and the total content of the ester-based ashless friction modifier (C1) and the amine-based ashless friction modifier (C2) is more than 0.1 mass% and 1.8 mass% or less based on the total amount of the lubricating oil composition.

In a case where the total content of the ester-based ashless friction modifier (C1) and the amine-based ashless friction modifier (C2) is 0.1 mass% or less based on the total amount of the lubricating oil composition, it is not possible to impart a friction-reducing effect based on the component (C1) and/or the component (C2). Further, in a case where the total content of the ester-based ashless friction modifier (C1) and the amine-based ashless friction modifier (C2) is more than 1.8 mass% based on the total amount of the lubricating oil composition, a friction-reducing effect based on the molybdenum compound (B) is inhibited, and in turn, the friction coefficient increases.

Meanwhile, by allowing the lubricating oil composition of the present embodiment to use the ester-based ashless friction modifier (C1) and the amine-based ashless friction modifier (C2) as the ashless friction modifier of the component (C), and allowing the total content of these components to fall within the range, the lubricating oil composition can enhance the friction-reducing effect, and thus enhance the fuel consumption reducing properties.

The total content of the ester-based ashless friction modifier (C1) and the amine-based ashless friction modifier (C2) is preferably 0.2 mass% or more and 1.7 mass% or less, and more preferably 0.4 mass% or more and 1.6 mass% or less, based on the total amount of the lubricating oil composition.

### Ester-Based Ashless Friction Modifier (C 1)

Various ester compounds can be used as the ester-based ashless friction modifier of the component (C1), in which an ester compound having one or more hydroxyl groups in a molecule thereof is preferable, and an ester compound having two or more hydroxyl groups in a molecule thereof is more preferable.

In addition, the ester compound having one or more hydroxyl groups in a molecule thereof preferably has 2 to 24 carbon atoms, more preferably has 10 to 24 carbon atoms, and still more preferably has 16 to 22 carbon atoms.

Examples of the ester compound having one or more hydroxyl groups in a molecule thereof include an ester compound having one hydroxyl group in a molecule thereof as in the following general formula (II) and a compound having two hydroxyl groups in a molecule thereof as in the following general formula (III). Among these, a compound represented by the general formula (III) is suitable.

In the general formulae (II) and (III), R⁵ and R¹⁰ are each a hydrocarbon group having 1 to 32 carbon atoms.

The number of carbon atoms of the hydrocarbon group of R⁵ and R¹⁰ is preferably 8 to 32, more preferably 12 to 24, and still more preferably 16 to 20.

Examples of the hydrocarbon group of R⁵ and R¹⁰ include an alkyl group, an alkenyl group, an alkylaryl group, a cycloalkyl group, and a cycloalkenyl group. Among these, an alkyl group or an alkenyl group is preferable, with an alkenyl group being more preferable.

Examples of the alkyl group in R⁵ and R¹⁰ include a methyl group, an ethyl group, a propyl group, a butyl group, a pentyl group, a hexyl group, a heptyl group, an octyl group, a nonyl group, a decyl group, an undecyl group, a dodecyl group, a tridecyl group, a tetradecyl group, a pentadecyl group, a hexadecyl group, a heptadecyl group, an octadecyl group, a nonadecyl group, an eicosyl group, a heneicosyl group, a docosyl group, a tricosyl group, and a tetracosyl group. These may be linear, branched, or cyclic.

Furthermore, examples of the alkenyl group in R⁵ and R¹⁰ include a vinyl group, a propenyl group, a butenyl group, a pentenyl group, a hexenyl group, a heptenyl group, an octenyl group, a nonenyl group, a decenyl group, an undecenyl group, a dodecenyl group, a tridecenyl group, a tetradecenyl group, a pentadecenyl group, a hexadecenyl group, a heptadecenyl group, an octadecenyl group, a nonadecenyl group, an eicosenyl group, a heneicosenyl group, a docosenyl group, a tricosenyl group, and a tetracosenyl group. These may be linear, branched, or cyclic, and the position of the double bond is arbitrary.

R⁶ to R⁹ and R¹¹ to R¹⁵ are each a hydrogen atom or a hydrocarbon group having 1 to 18 carbon atoms, and they may be the same as or different from each other.

In the general formula (II), it is preferable that all of R⁶ to R⁹ are a hydrogen atom, or all of R⁶ to R⁸ are a hydrogen atom, and R⁹ is a hydrocarbon group. Further, in the general formula (III), it is preferable that all of R¹¹ to R¹⁵ are a hydrogen atom.

In a case where the compound represented by the general formula (II) is used as the ester-based ashless friction modifier (C1), a single kind of the compound in which all of R^{5'}s to R^{9'}s are all the same may be used, or a mixture of two or more kinds of the compounds in which some of R^{5'}s to R^{9'}s are different (for example, those in which the number of carbon atoms or the presence or absence of a double bond of R^{5'}s is different) may be used. Similarly, in a case where the compound represented by the general formula (III) is used as the ester-based ashless friction modifier (C 1), a single kind of the compound in which all of R^{10'}s to R^{15'}s are all the same may be used, or a mixture of two or more kinds of the compounds in which R^{10'}s to R^{15'}s are different (for example, those in which the number of carbon atoms or the presence or absence of a double bond of R^{10'}s is different, or R^{11'}s to R^{15'}s are different) may be used.

In a case where R⁶ to R⁹ and R¹¹ to R¹⁵ are a hydrocarbon group, the hydrocarbon group may be either saturated or unsaturated, may be either aliphatic or aromatic, and may be linear, branched, or cyclic.

Furthermore, in the general formula (II), "a" represents an integer of 1 to 20, and is preferably 1 to 12, and more preferably 1 to 10.

The compound represented by the general formula (II) is, for example, a compound obtained through a reaction of a fatty acid and an alkylene oxide.

Here, examples of the fatty acid for obtaining the compound represented by the general formula (II) include lauric acid, myristic acid, palmitic acid, oleic acid, tallow acid, and coconut fatty acid. Examples of the alkylene oxide include alkylene oxides having 2 to 12 carbon atoms, and specific examples thereof include ethylene oxide, propylene oxide, butylene oxide, hexylene oxide, octylene oxide, decylene oxide, and dodecylene oxide.

Examples of the compound of the general formula (II) include polyoxyethylene monolaurate, polyoxyethylene monostearate, and polyoxyethylene monooleate.

Examples of the compound represented by the general formula (III) include glycerin fatty acid monoesters such as glycerin monolaurate, glycerin monostearate, glycerin monomyristate, and glycerin monooleate. Among these, glycerin monooleate is suitable.

### Amine-Based Ashless Friction Modifier (C2)

As the amine-based ashless friction modifier (C2), an aliphatic amine-based compound having one or more hydroxyl groups in a molecule thereof is used. Further, the amine-based ashless friction modifier (C2) may be any one of primary, secondary, and tertiary amines, with a tertiary amine being suitable.

Examples of the amine-based ashless friction modifier (C2) which is a tertiary amine, as the aliphatic amine-based compound having one or more hydroxyl groups in a molecule thereof, include compounds represented by the following general formulae (IV) and (V), with a compound represented by the general formula (IV) being suitable.

In the general formulae (IV) and (V), R¹⁶, R²⁵, and R²⁶ are each a hydrocarbon group having 1 to 32 carbon atoms, and R²⁵ and R²⁶ may be the same as or different from each other.

The number of carbon atoms of the hydrocarbon group of R¹⁶, R²⁵, and R²⁶ is preferably 8 to 32, more preferably 10 to 24, and still more preferably 12 to 20.

Examples of the hydrocarbon group of R¹⁶, R²⁵, and R²⁶ include an alkyl group, an alkenyl group, an alkylaryl group, a cycloalkyl group, and a cycloalkenyl group. Among these, an alkyl group or an alkenyl group is preferable.

Examples of the alkyl group of R¹⁶, R²⁵, and R²⁶ include a methyl group, an ethyl group, a propyl group, a butyl group, a pentyl group, a hexyl group, a heptyl group, an octyl group, a nonyl group, a decyl group, an undecyl group, a dodecyl group, a tridecyl group, a tetradecyl group, a pentadecyl group, a hexadecyl group, a heptadecyl group, an octadecyl group, a nonadecyl group, an eicosyl group, a heneicosyl group, a docosyl group, a tricosyl group, and a tetracosyl group. These may be linear, branched, or cyclic.

Furthermore, examples of the alkenyl group represented by R¹⁶, R²⁵, and R²⁶ include a vinyl group, a propenyl group, a butenyl group, a pentenyl group, a hexenyl group, a heptenyl group, an octenyl group, a nonenyl group, a decenyl group, an undecenyl group, a dodecenyl group, a tridecenyl group, a tetradecenyl group, a pentadecenyl group, a hexadecenyl group, a heptadecenyl group, an octadecenyl group, a nonadecenyl group, an eicosenyl group, a heneicosenyl group, a docosenyl group, a tricosenyl group, and a tetracosenyl group. These may be linear, branched, or cyclic, and the position of the double bond is arbitrary.

R¹⁷ to R²⁴ and R²⁷ to R³⁰ are each a hydrogen atom, a hydrocarbon group having 1 to 18 carbon atoms, or an oxygen-containing hydrocarbon group that contains an ether bond or an ester bond. These may be the same as or different from each other, and each is preferably a hydrogen atom or the hydrocarbon group.

The hydrocarbon group of R¹⁷ to R²⁴ and R²⁷ to R³⁰ may be saturated or unsaturated, aliphatic or aromatic, and linear, branched or cyclic, and examples of the hydrocarbon group include aliphatic hydrocarbon groups such as an alkyl group and an alkenyl group, and aromatic hydrocarbon groups. More specific examples thereof include aliphatic hydrocarbon groups such as a methyl group, an ethyl group, a propyl group, a butyl group, a butenyl group, a hexyl group, a hexenyl group, an octyl group, an octenyl group, a 2-ethylhexyl group, a nonyl group, a decyl group, an undecyl group, a decenyl group, a dodecyl group, a dodecenyl group, a tridecyl group, a tetradecyl group, a tetradecenyl group, a pentadecyl group, a hexadecyl group, a hexadecenyl group, a heptadecyl group, an octadecyl group, an octadecenyl group, a stearyl group, an isostearyl group, an oleyl group, a linoleic group, a cyclopentyl group, a cyclohexyl group, a methylcyclohexyl group, an ethylcyclohexyl group, a propylcyclohexyl group, a dimethylcyclohexyl group, and a trimethylcyclohexyl group; and aromatic hydrocarbon groups such as a phenyl group, a methylphenyl group, an ethylphenyl group, a dimethylphenyl group, a propylphenyl group, a trimethylphenyl group, a butylphenyl group, and a naphthyl group.

The hydrocarbon group is preferably a hydrocarbon group having 1 to 18 carbon atoms, more preferably a hydrocarbon group having 1 to 12 carbon atoms, still more preferably a hydrocarbon group having 1 to 4 carbon atoms, and most preferably a hydrocarbon group having 2 carbon atoms.

The oxygen-containing hydrocarbon group that contains an ether bond or an ester bond is preferably the group having 1 to 18 carbon atoms, and examples thereof include a methoxymethyl group, an ethoxymethyl group, a propoxymethyl group, an isopropoxymethyl group, a n-butoxymethyl group, a t-butoxymethyl group, a hexyloxymethyl group, an octyloxymethyl group, a 2-ethyl-hexyloxymethyl group, a decyloxymethyl group, a dodecyloxymethyl group, a 2-butyloctyloxymethyl group, a tetradecyloxymethyl group, a hexadecyloxymethyl group, a 2-hexyldodecyloxymethyl group, an allyloxymethyl group, a phenoxy group, a benzyloxy group, a methoxyethyl group, a methoxypropyl group, a 1,1-bismethoxypropyl group, a 1,2-bismethoxypropyl group, an ethoxypropyl group, a (2-methoxyethoxy)propyl group, a (1-methyl-2-methoxy)propyl group, an acetyloxymethyl group, a propanoyloxymethyl group, a butanoyloxymethyl group, a hexanoyloxymethyl group, an octanoyloxymethyl group, a 2-ethylhexanoyloxymethyl group, a decanoyloxymethyl group, a dodecanoyloxymethyl group, a 2-butyloctanoyloxymethyl group, a tetradecanoyloxymethyl group, a hexadecanoyloxymethyl group, a 2-hexyldodecanoyloxymethyl group, and a benzoyloxymethyl group.

Furthermore, b to d each represents an integer of 0 to 20.

b + c is preferably 1 to 20, more preferably 1 to 10, still more preferably 1 to 4, and most preferably 2.

In the general formula (IV), it is preferable that all of R¹⁷ to R²⁴ are a hydrogen atom. Further, in the general formula (V), it is preferable that all of R²⁷ to R³⁰ are a hydrogen atom.

In a case where the aliphatic amine compound of the general formula (IV) is used as the amine-based ashless friction modifier (C2), the aliphatic amine compounds in which all of R^{16'}s are all the same may be used, or a mixture of the aliphatic amine compounds in which R^{16'}s are different (for example, those in which the number of carbon atoms or the presence or absence of a double bond is different) as for naturally derived hydrocarbon groups such as beef tallow may be used. Similarly, in the case where the aliphatic amine compound of the general formula (V) is used as the amine-based ashless friction modifier (C2), the aliphatic amine compounds in which R^{25'}s and R^{26'}s are all the same may be used, or a mixture of the aliphatic amine compounds in which R^{25'}s and R^{26'}s are different (for example, those in which the number of carbon atoms or the presence or absence of a double bond is different) may be used.

Specific examples of the compounds of the general formula (IV) include amine compounds having one 2-hydroxyalkyl group, for example, a hydroxyethyl group, such as octyl ethanolamine, decyl ethanolamine, dodecyl ethanolamine, tetradecyl ethanolamine, hexadecyl ethanolamine, stearyl ethanolamine, oleyl ethanolamine, coconut oil ethanolamine, palm oil ethanolamine, rapeseed oil ethanolamine, and beef tallow ethanolamine; amine compounds having two 2-hydroxyalkyl groups, such as octyl diethanolamine, decyl diethanolamine, dodecyl diethanolamine, tetradecyl diethanolamine, hexadecyl diethanolamine, stearyl diethanolamine, oleyl diethanolamine, coconut oil diethanolamine, palm oil diethanolamine, rapeseed oil diethanolamine, and beef tallow diethanolamine; and amine compounds having a polyalkylene oxide structure, such as polyoxyethylene octylamine, polyoxyethylene decylamine, polyoxyethylene dodecylamine, polyoxyethylene tetradecylamine, polyoxyethylene hexadecylamine, polyoxyethylene stearylamine, polyoxyethylene oleylamine, polyoxyethylene beef tallow amine, polyoxyethylene coconut oil amine, polyoxyethylene palm oil amine, polyoxyethylene laurylamine, polyoxyethylene stearylamine, polyoxyethylene oleylamine, and ethylene oxide-propylene oxide stearylamine.

Specific examples of the compounds of the general formula (V) include alkylamine compounds having one 2-hydroxyalkyl group, for example, hydroxyethyl groups such as N-methyl-octyl ethanolamine, N-methyl-decyl ethanolamine, N-methyl-dodecyl ethanolamine, N-methyl-tetradecyl ethanolamine, N-methyl-hexadecyl ethanolamine, N-methyl-stearyl ethanolamine, N-methyl-oleyl ethanolamine, N-methyl-coconut oil ethanolamine, N-methyl-palm oil ethanolamine, N-methyl-rapeseed oil ethanolamine, and N-methyl-beef tallow ethanolamine; and alkylamine compounds having a polyalkylene oxide structure, such as polyoxyethylene N-methyl-decylamine, polyoxyethylene N-methyl-dodecylamine, polyoxyethylene N-methyl-tetradecylamine, polyoxyethylene N-methyl-hexadecylamine, polyoxyethylene N-methyl-stearylamine, and polyoxyethylene N-methyl-oleylamine.

The lubricating oil composition of the present embodiment may include any one of the ester-based ashless friction modifier (C1) and the amine-based ashless friction modifier (C2) as the ashless friction modifier of the component (C), and the ester-based ashless friction modifier (C1) is used in combination with the amine-based ashless friction modifier (C2).

By using the ester-based ashless friction modifier (C1) in combination with the amine-based ashless friction modifier (C2), a friction-reducing effect based on the molybdenum compound (B) can be more easily maintained. That is, by using the ester-based ashless friction modifier (C1) in combination with the amine-based ashless friction modifier (C2), it is possible to impart a friction-reducing effect based on three components of the molybdenum compound (B), the ester-based ashless friction modifier (C1), and the amine-based ashless friction modifier (C2), and thus, fuel consumption reducing properties can be more improved.

Furthermore, from the viewpoint that the effect can be easily exhibited by using the ester-based ashless friction modifier (C1) in combination with the amine-based ashless friction modifier (C2), the mass ratio of the content of the amine-based ashless friction modifier (C2) to the content of the ester-based ashless friction modifier (C1) [the content of the amine-based ashless friction modifier (C2)/the content of the ester-based ashless friction modifier (C1)] is 0.15 or more and 0.80 or less, and preferably 0.15 or more and 0.60 or less.

Moreover, the mass ratio of the total content of the ester-based ashless friction modifier (C1) and the amine-based ashless friction modifier (C2) to the content of the molybdenum compound (B) as converted into molybdenum atoms [(the content of the ester-based ashless friction modifier (C1) + the content of the amine-based ashless friction modifier (C2))/the content of the molybdenum compound (B) as converted into molybdenum atoms] is preferably 4.0 to 30.0, more preferably 5.0 to 25.0, and still more preferably 6.5 to 23.0.

The ashless friction modifier (C) may contain ashless type friction modifiers (other ashless type friction modifiers) other than the ester-based ashless friction modifier (C 1) and the amine-based ashless friction modifier (C2), within a range not impairing the effect of the lubricating oil composition of the present embodiment. Here, the total content of the ester-based ashless friction modifier (C1) and the amine-based ashless friction modifier (C2) based on the total amount of the ashless friction modifier (C), is preferably 80 mass% or more, more preferably 90 mass% or more, and still more preferably 100 mass%.

### <Borated succinimide (D)>

The lubricating oil composition of the present embodiment preferably further includes a borated succinimide (D).

By using the molybdenum compound (B), and the ester-based ashless friction modifier (C1) and/or the amine-based ashless friction modifier (C2), together with the borated succinimide (D), a friction-reducing effect based on the molybdenum compound (B) can be more easily maintained, and as a result, the synergistic action with the molybdenum compound (B) and the ester-based ashless friction modifier (C1) and/or the amine-based ashless friction modifier (C2) is easily exhibited, the friction-reducing effect is more enhanced, and the fuel consumption reducing properties can be enhanced.

Examples of the borated succinimide of the component (D) include boronated products of alkenyl- or alkylsuccinic monoimide, or boronated products of alkenyl- or alkylsuccinic bisimide.

Examples of the alkenyl- or alkylsuccinic monoimide include a compound represented by the following general formula (VI). Further, examples of the alkenyl- or alkylsuccinic bisimide include a compound represented by the following general formula (VII).

In the general formulae (VI) and (VII), R³¹, R³³, and R³⁴ are each an alkenyl group or an alkyl group, and they each have a weight average molecular weight of preferably 500 to 3,000, and more preferably 1,000 to 3,000.

If the weight average molecular weight of R³¹, R³³, and R³⁴ is 500 or more, the solubility in a lubricating base oil can be enhanced. Further, if the weight average molecular weight is 3,000 or less, it is expected that the effect obtained by the present compound is appropriately exhibited. R³³ and R³⁴ may be the same as or different from each other.

R³², R³⁵, and R³⁶ are each an alkylene group having 2 to 5 carbon atoms, and R³⁵ and R³⁶ may be the same as or different from each other. "e" represents an integer of 1 to 10, and "f" represents 0 or an integer of 1 to 10.

Here, "e" is preferably 2 to 5, and more preferably 2 to 4. If "e" is 2 or more, it is expected that the effect obtained by the borated succinimide is easily obtained. If "e" is 5 or less, the solubility in a lubricating base oil is more enhanced.

Furthermore, "f" is preferably 1 to 6, and more preferably 2 to 6. If "f" is 1 or more, it is expected that the effect obtained by the present compound is appropriately exhibited. If "f" is 6 or less, the solubility in a lubricating base oil is enhanced.

Examples of the alkenyl group include a polybutenyl group, a polyisobutenyl group, and an ethylene-propylene copolymer, and examples of the alkyl group include hydrogenated products thereof. Suitable examples of the alkenyl group include a polybutenyl group and a polyisobutenyl group. As the polybutenyl group, a mixture of 1-butene and isobutene or a product obtained by polymerization of high-purity isobutene is suitably used. Further, suitable representative examples of the alkyl group include hydrogenated products of a polybutenyl group or a polyisobutenyl group.

The borated succinimide (D) can be obtained by, for example, reacting a polyolefin with maleic anhydride to obtain an alkenylsuccinic anhydride (x); reacting a polyamine with a boron compound to obtain an intermediate (y); and then reacting the alkenylsuccinic anhydride (x) with the intermediate (y), followed by imidization. The monoimide or the bisimide can be produced by changing the ratio of the alkenylsuccinic anhydride or the alkylsuccinic anhydride to the polyamine.

In addition, the borated succinimide (D) can also be produced by treating an alkenyl- or alkylsuccinic monoimide or an alkenyl- or alkylsuccinic bisimide not containing boron with the boron compound.

As the olefin monomer that forms the polyolefin, one kind or a mixture of two or more kinds of α-olefins having 2 to 8 carbon atoms can be used, but a mixture of isobutene and 1-butene can be suitably used.

Meanwhile, examples of the polyamine include single diamines such as ethylenediamine, propylenediamine, butylendiamine, and pentylenediamine; polyalkylene polyamines such as diethylenetriamine, triethylenetetramine, tetraethylenepentamine, pentaethylenehexamine, di(methylethylene)triamine, dibutylentriamine, tributylentetramine, and pentapentylenehexamine; and piperazine derivatives such as aminoethylpiperazine.

Examples of the boron compound include boric acid, borate, and a boric acid ester.

Examples of the boric acid include orthoboric acid, metaboric acid, and paraboric acid. Further, examples of the borate include ammonium borate, such as ammonium metaborate, ammonium tetraborate, ammonium pentaborate, and ammonium octaborate. Further, examples of the boric acid ester include monomethyl borate, dimethyl borate, trimethyl borate, monoethyl borate, diethyl borate, triethyl borate, monopropyl borate, dipropyl borate, tripropyl borate, monobutyl borate, dibutyl borate, and tributyl borate.

The ratio (B/N ratio) of the amount of boron atoms to the amount of nitrogen atoms, which are contained in the borated succinimide (D), is preferably 0.6 or more, more preferably 0.7 or more, and still more preferably 0.8 or more, on a mass basis, in terms of friction reduction. Further, the B/N ratio is not particularly limited, but is preferably 2.0 or less, more preferably 1.5 or less, and still more preferably 1.3 or less.

From the viewpoint of friction reduction, the borated succinimide (D) preferably includes a large amount of a three-coordinate borated succinimide, and specifically, includes a three-coordinate borated succinimide at a molar ratio of preferably 0.50 or more, more preferably 0.60 or more, and still more preferably 0.65 or more, relative to the total amount of three-coordinate borated succinimide and four-coordinate borated succinimide.

The ratio of three-coordinate borated succinimide and the four-coordinate borated succinimide can be measured by, for example, ¹¹B-NMR measurement as a BF₃·OEt₂ standard (0 ppm). In this ¹¹B-NMR measurement, the peaks of the three-coordinate borated succinimide are shown at 5 to 25 ppm, and the peaks of the four-coordinate borated succinimide are shown at -10 to 5 ppm, and thus, it is possible to calculate the ratio by calculating the integrated value of the respective peaks.

Moreover, in the lubricating oil composition of the present embodiment, the content of the borated succinimide (D) as converted into boron atoms is preferably 0.050 mass% or less, more preferably 0.001 to 0.050 mass%, still more preferably 0.005 to 0.040 mass%, and even still more preferably 0.015 to 0.035 mass%, based on the total amount of the lubricating oil composition.

By allowing the content of the borated succinimide (D) as converted into boron atoms to fall within the range, inhibition of a friction-reducing effect based on the molybdenum compound (B) can be suppressed, and as a result, the synergistic action with the molybdenum compound (B), and the ester-based ashless friction modifier (C1) and/or the amine-based ashless friction modifier (C2) can be more exhibited, the friction-reducing effect can be more enhanced, and thus, the fuel consumption reducing properties can be more improved.

Furthermore, in the lubricating oil composition of the present embodiment, the mass ratio of the content of the borated succinimide (D) as converted into boron atoms to the total content of the ester-based ashless friction modifier (C1) and the amine-based ashless friction modifier (C2) [the content of the borated succinimide (D) as converted into boron atoms/(the content of the ester-based ashless friction modifier (C1) + the content of the amine-based ashless friction modifier (C2))] is preferably 0.011 or more, more preferably 0.013 or more and 0.100 or less, and still more preferably 0.015 or more and 0.070 or less.

By allowing the ratio to fall within the range, inhibition of a friction-reducing effect based on the molybdenum compound (B) can be more suppressed, and by the synergistic action with the molybdenum compound (B) and the ester-based ashless friction modifier (C1), the friction-reducing effect is more enhanced, and thus, the fuel consumption reducing properties can be more improved.

### <Poly(meth)acrylate (E)>

It is preferable that the lubricating oil composition of the present embodiment further contains a poly(meth)acrylate (E) as a viscosity index improver. By containing the poly(meth)acrylate (E), the fuel consumption reducing properties can be more improved.

The monomer constituting the poly(meth)acrylate (E) is alkyl (meth)acrylate, and preferably alkyl (meth)acrylate with a linear alkyl group having 1 to 18 carbon atoms or a branched alkyl group having 3 to 34 carbon atoms.

Preferred examples of the monomer constituting the poly(meth)acrylate (E) include methyl (meth)acrylate, ethyl (meth)acrylate, propyl (meth)acrylate, butyl (meth)acrylate, pentyl (meth)acrylate, hexyl (meth)acrylate, hexyl (meth)acrylate, heptyl (meth)acrylate, octyl (meth)acrylate, nonyl (meth)acrylate, decyl (meth)acrylate, dodecyl (meth)acrylate, tetra(meth)acrylate, hexa(meth)acrylate, and octadecyl (meth)acrylate, and two or more kinds of these monomers may be used as a copolymer. The alkyl group of these monomers may be linear chained or branch chained.

Furthermore, examples of the alkyl (meth)acrylate with a branched alkyl group having 3 to 34 carbon atoms include isopropyl (meth)acrylate, 2-ethylhexyl (meth)acrylate, 3,5,5-trimethylhexyl (meth)acrylate, 2-butyloctyl (meth)acrylate, 2-hexyldecyl (meth)acrylate, 2-octyldodecyl (meth)acrylate, 2-decyltetradecyl (meth)acrylate, 2-dodecyl hexadecyl (meth)acrylate, and 2-tetradecyloctadecyl (meth) acrylate.

The weight average molecular weight of the poly(meth)acrylate (E) is preferably 100,000 to 600,000, and more preferably 15,000 to 400,000.

Moreover, in the present embodiment, the "weight average molecular weight" refers to a molecular weight as converted into polystyrene, which is determined by a gel permeation chromatography (GPC) measurement.

The SSI of the poly(meth)acrylate (E) is preferably 50 or less, and more preferably 1 to 30. By allowing the weight average molecular weight to fall within the above range, the SSI can be adjusted to 30 or less.

Here, the SSI means a shear stability index, and represents an ability of resisting to decomposition of a poly(meth)acrylate. As the SSI is larger, the polymer is more unstable against shear and more easily decomposes. The SSI indicates a decrease in viscosity under shear derived from a polymer, and is calculated using the above calculation equation. In the equation, Kv₀ represents a value of kinematic viscosity at 100°C of a mixture obtained by adding a poly(meth)acrylate to a base oil. Kv₁ is a value of kinematic viscosity at 100°C measured after passing the mixture obtained by the addition of poly(meth)acrylate to the base oil through a high-shear Bosch diesel injector for 30 cycles in accordance with the procedures of ASTM D6278. Further, Kvₒᵢₗ is a value of kinematic viscosity at 100°C of the base oil. In addition, as the base oil, a Group II base oil having a kinematic viscosity at 100°C of 5.35 mm²/s and a viscosity index of 105 is used.

From the viewpoint of fuel consumption reducing properties, the content of the poly(meth)acrylate (E) is preferably 0.5 to 15 mass%, more preferably 1 to 10 mass%, and still more preferably 1 to 8 mass%, based on the total amount of the lubricating oil composition.

Here, the content of the poly(meth)acrylate means the content of only the resin fractions composed of poly(meth)acrylate, and is, for example, a content on a solid content basis which does not include the mass of a diluent oil and the like which are contained together with the poly(meth)acrylate.

### <Metal-Based Detergent (F)>

It is preferable that the lubricating oil composition of the present embodiment further contains a metal-based detergent (F). By containing the metal-based detergent (F), production of a deposit in the inside of an engine at the time of high-temperature operation is suppressed, accumulation of a sludge is prevented to keep the inside of the engine clean, and acidic substance generated as a result of degradation and the like of an engine oil is neutralized to prevent corrosive wear.

Examples of the metal-based detergent (F) include an alkali metal-based detergent or an alkaline-earth metal-based detergent. Specific examples thereof include one or more metal-based detergents selected from alkali metal sulfonate or alkaline-earth metal sulfonate, alkali metal phenate or alkaline-earth metal phenate, alkali metal salicylate, or alkaline-earth metal salicylate. Further, examples of the alkali metal include sodium and potassium, examples of the alkaline-earth metal include magnesium and calcium, and among these, sodium which is an alkali metal, and magnesium and calcium which are alkaline-earth metals are preferable, and calcium is more preferable.

The metal-based detergent (F) may be neutral, basic, or overbasic, but is preferably basic or overbasic. Further, the total base number of the metal-based detergent (F) is preferably 10 to 500 mgKOH/g, and more preferably 150 to 450 mgKOH/g. Further, the total base number is one as measured in accordance with a perchloric acid method of JIS K2501.

From the viewpoint of exhibiting an effect based on the above-mentioned metal-based detergent (F), the content of the metal-based detergent (F) as converted into a metal amount in the lubricating oil composition of the present embodiment is preferably 0.05 to 0.50 mass%, and more preferably 0.10 to 0.30 mass%, based on the total amount of the lubricating oil composition.

### <Zinc Dithiophosphate (G)>

It is preferable that the lubricating oil composition of the present embodiment further contains zinc dithiophosphate (G). By containing zinc dithiophosphate of the component (G), the friction-reducing effect can be more enhanced.

Examples of the zinc dithiophosphate (G) include those represented by the following general formula (VIII): in the formula, R³⁷ to R⁴⁰ each independently represents any one selected from a linear, branched, or cyclic alkyl group having 6 to 20 carbon atoms, and a linear, branched, or cyclic alkenyl group having 6 to 20 carbon atoms.

By allowing the number of carbon atoms of R³⁷ to R⁴⁰ in the general formula (VIII) to be 6 to 20, a balance between the solubility in a lubricating base oil and the friction reduction can be enhanced.

The number of carbon atoms of the alkyl group or the alkenyl group of R³⁷ to R⁴⁰ in the general formula (VIII) is preferably 8 to 18, and more preferably 10 to 14. Further, R³⁷ to R⁴⁰ in the general formula (VIII) are each preferably an alkyl group.

Examples of the alkyl group in R³⁷ to R⁴⁰ include a methyl group, an ethyl group, a propyl group, a butyl group, a pentyl group, a hexyl group, a heptyl group, an octyl group, a nonyl group, a decyl group, an undecyl group, a dodecyl group, a tridecyl group, a tetradecyl group, a pentadecyl group, a hexadecyl group, a heptadecyl group, an octadecyl group, a nonadecyl group, an eicosyl group, a heneicosyl group, a docosyl group, a tricosyl group, and a tetracosyl group, and these may be linear, branched, or cyclic. Further, examples of the alkenyl group include a vinyl group, a propenyl group, a butenyl group, a pentenyl group, a hexenyl group, a heptenyl group, an octenyl group, a nonenyl group, a decenyl group, an undecenyl group, a dodecenyl group, a tridecenyl group, a tetradecenyl group, a pentadecenyl group, a hexadecenyl group, a heptadecenyl group, an octadecenyl group, a nonadecenyl group, an eicosenyl group, a heneicosenyl group, a docosenyl group, a tricosenyl group, and a tetracosenyl group. These may be linear, branched, or cyclic, and the position of the double bond is arbitrary.

In the general formula (VIII), R³⁷ to R⁴⁰ may be the same as or different from each other, and from the viewpoint of easiness in terms of production, they are preferably the same as each other.

Among these, dodecyl groups such as a lauryl group, octadecyl groups such as a tetradecyl group, a hexadecyl group, and a stearyl group, and octadecenyl groups such as an eicosyl group and an oleyl group are preferable, and a lauryl group is the most preferable.

From the viewpoint of a balance between friction reduction and abrasion resistance, the content of zinc dithiophosphate (G) is preferably 0.01 to 3.00 mass%, and more preferably 0.10 to 1.50 mass%, based on the total amount of the lubricating oil composition.

Furthermore, the content of zinc dithiophosphate (G) as converted into phosphorus atoms is preferably 100 to 2,000 ppm, more preferably 300 to 1,500 ppm, still more preferably 500 to 1,000 ppm, and even still more preferably 600 to 840 ppm, based on the total amount of the lubricating oil composition.

### <Arbitrary Additive Components>

The lubricating oil composition of the present embodiment may contain arbitrary additive components such as succinimide not containing boron, an antioxidant, a rust inhibitor, a metal deactivator, a pour-point depressant, and an antifoaming agent as arbitrary components.

The content of these arbitrary additive components is approximately 0.01 to 5.00 mass% based on the total amount of the lubricating oil composition.

### <Physical Properties of Lubricating Oil Composition>

From the viewpoint of friction reduction over a wide temperature range from a low temperature to a high temperature, it is preferable that the lubricating oil composition of the present embodiment has a kinematic viscosity at 40°C, a kinematic viscosity at 100°C, and an HTHS viscosity at 150°C, each of which falls within the following range.

The kinematic viscosity at 40°C is preferably 20 to 40 mm²/s, and more preferably 20 to 35 mm²/s.

The kinematic viscosity at 100°C is preferably 3.0 to 12.5 mm²/s, and more preferably 4.0 to 9.3 mm²/s.

The HTHS viscosity at 150°C is preferably 1.4 to 2.9 mPa s, and more preferably 1.7 to 2.9 mPa s.

Furthermore, the kinematic viscosity was measured in conformity with JIS K2283. The HTHS viscosity was measured using a TBS viscometer (tapered bearing simulator viscometer) in accordance with ASTM D4683 under the conditions at an oil temperature of 100°C, a shear rate of 10⁶/s, a rotational speed (motor) of 3,000 rpm, and a clearance (clearance between a rotor and a stator) of 3 µm.

### <Application of Lubricating Oil Composition>

The lubricating oil composition of the present embodiment is not particularly limited with respect to its application, but it can be suitably used for a variety of internal combustion engines of a four-wheel automobile, a two-wheel automobile, or the like. Further, among the internal combustion engines, the lubricating oil composition of the present embodiment can be particularly suitably used for a gasoline engine.

### [Method for Reducing Friction of Internal Combustion Engine]

The method for reducing friction of an internal combustion engine of the present embodiment includes adding the above-mentioned lubricating oil composition of the present embodiment to an internal combustion engine.

According to the method for reducing friction of an internal combustion engine of the present embodiment, inhibition of a friction-reducing effect based on the molybdenum compound (B) is suppressed; and by the synergistic action with the molybdenum compound (B), and the ester-based ashless friction modifier (C1) and/or the amine-based ashless friction modifier (C2), the friction-reducing effect is enhanced, and thus, the fuel consumption reducing properties can be enhanced. In a case where the internal combustion engine is a gasoline engine, the effect can be particularly enhanced.

### EXAMPLES

Next, the present invention will be described in more detail with reference to Examples, but it should be construed that the present invention is by no means limited by these Examples.

### 1. Preparation of Lubricating Oil Compositions of Examples and Comparative Examples

Lubricating oil compositions of Examples and Comparative Examples were prepared in the compositions shown in Tables 1 to 3. Further, for the preparation of the lubricating oil compositions, the following materials were used.

### <Lubricating Base Oil (A)>

Mineral oil having a kinematic viscosity at 100°C: 4.07 mm²/s, viscosity index: 131, %C_{A}: -0.4, %C_{N}: 12.8, and %C_{P}: 87.6

### <Molybdenum Compound (B)>

Binuclear organic molybdenum compound of the general formula (I) (MoDTC having an Mo content of 10 mass%)

### <Ester-Based Ashless Friction Modifier (C1)>

Glycerin monooleate (number of hydroxyl groups in one molecule: 2)

### <Amine-Based Ashless Friction Modifier (C2)>

Alkyldiethanolamine (the number of carbon atoms of an alkyl group being a mixture of 12 to 20)

### <Borated succinimide (D)>

Borated polybutenylsuccinic bisimide (boron content: 1.3 mass%, nitrogen content: 1.2 mass%, amount of boron atoms/amount of nitrogen atoms: 1.1)

### <Poly(meth)acrylate (E)>

Polymethacrylate (weight average molecular weight of 440,000, content of the resin fraction of 17%, SSI of 30)

### <Metal-Based Detergent (F)>

Calcium-based detergent (calcium content: 12.1 mass%, overbasic, total base number: 350 mgKOH/g)

### <Zinc Dithiophosphate (G)>

ZnDTP (phosphorus content: 7.0 mass%, zinc content: 8.0 mass%, sulfur content: 14.0 mass%)

### <Other Components>

Polybutenylsuccinic bisimide which is not a borated material, a hindered phenol-based antioxidant, a diphenylamine-based antioxidant, a pour-point depressant, a metal deactivator, and an antifoaming agent

### 2. Measurement and Evaluation

The lubricating oil compositions of Examples and Comparative Examples which had been prepared in the compositions shown in Tables 1 to 3 were subjected to the following evaluations. The results are shown in Tables 1 to 3.

### 2-1. HTHS Viscosity

In accordance with the disclosure of the present specification, the HTHS viscosity at 150°C of the lubricating oil composition was measured.

### 2-2. Friction Coefficient (HFRR Test)

Using an HFRR tester (manufactured by PCS Instruments), the friction coefficient of the lubricating oil composition was measured under the following conditions. A lower friction coefficient may indicate that the friction-reducing effect is superior and the fuel consumption reducing properties are better.
- Test piece: (A) Ball=HFRR standard test piece (AISI 52100 material), (B) Disc =HFRR standard test piece (AISI 52100 material)
- Amplitude: 1.0 mm
- Frequency: 50 Hz
- Load: 5 g
- Temperature: 80°C

In Tables 1 to 3, [mass% of Mo] represents the content of the molybdenum compound (B) as converted into molybdenum atoms based on the total amount of the lubricating oil composition; [mass% of B] represents the content of the borated succinimide (D) as converted into boron atoms based on the total amount of the lubricating oil composition; and [mass% of Metal] represents the content of the metal-based detergent (F) as converted into metal atoms (calcium atoms) based on the total amount of the lubricating oil composition.
The examples marked with "*" are reference examples.

**Table 1**

| | | | Example 1* | Example 2* | Comparative Example 1 | Comparative Example 2 |
|---|---|---|---|---|---|---|
| Composition | Lubricating base oil (A) | mass% | Balance | Balance | Balance | Balance |
| | Molybdenum compound (B) | mass% | 0.7 | 0.7 | 0.7 | 0.7 |
| | Ester-based friction modifier (C1) | mass% | 0.5 | - | - | - |
| | Amine-based friction modifier (C2) | mass% | - | 0.5 | - | 2.0 |
| | Borated succinimide (D) | mass% | 2.3 | 2.3 | 2.3 | 2.3 |
| | Poly(meth)acrylate (E) | mass% | 10.3 | 10.3 | 10.3 | 10.3 |
| | Metal-based detergent (F) | mass% | 1.65 | 1.65 | 1.65 | 1.65 |
| | Zinc dithiophosphate (G) | mass% | 1.14 | 1.14 | 1.14 | 1.14 |
| | Other components | mass% | 6.16 | 6.16 | 6.16 | 6.16 |
| Properties of lubricating oil composition | Content of molybdenum derived from (B) | mass% of Mo | 0.070 | 0.070 | 0.070 | 0.070 |
| | Content of boron derived from (D) | mass% of B | 0.030 | 0.030 | 0.030 | 0.030 |
| | Content of metal derived from (F) | mass% of metal | 0.200 | 0.200 | 0.200 | 0.200 |
| | HTHS viscosity at 150°C | mPa·s | 2.6 | 2.6 | 2.6 | 2.6 |
| Evaluation | Friction coefficient | - | 0.057 | 0.057 | 0.065 | 0.109 |

As is clear from the results of Table 1, it can be confirmed that the lubricating oil compositions of Examples 1 and 2, each including the molybdenum compound (B), and a specific amount of the ester-based ashless friction modifier (C1) and/or the amine-based ashless friction modifier (C2), exhibit a better friction-reducing effect, as compared with the lubricating oil composition of Comparative Example 1, not including the ester-based ashless friction modifier (C1) and/or the amine-based ashless friction modifier (C2).

It can also be confirmed that the lubricating oil composition of Comparative Example 2, including more than an appropriate amount of the ester-based ashless friction modifier (C1) and/or the amine-based ashless friction modifier (C2) does not exhibit a good friction-reducing effect. The reason for this may be thought to be that the friction-reducing effect of the molybdenum compound (B) is inhibited by a large amount of the ester-based ashless friction modifier (C1) and/or the amine-based ashless friction modifier (C2).

**Table 2**

| | | | Example | | | | | | | Comparative Example 3 |
|---|---|---|---|---|---|---|---|---|---|---|
| | | | 3* | 4* | 5* | 6 | 7 | 8 | 9* | |
| Composition | Lubricating base oil (A) | mass% | Balance | Balance | Balance | Balance | Balance | Balance | Balance | Balance |
| | Molybdenum compound (B) | mass% | 0.7 | 0.7 | 0.7 | 0.7 | 0.3 | 0.7 | 0.7 | 0.7 |
| | Ester-based friction modifier (C1) [X] | mass% | 1.0 | - | 1.0 | 0.5 | 0.5 | 1.0 | 0.5 | 2.0 |
| | Amine-based friction modifier (C2) [Y] | mass% | - | 0.5 | 0.1 | 0.1 | 0.1 | 0.5 | 0.5 | 0.5 |
| | Borated succinimide (D) | mass% | 2.3 | 2.3 | 2.3 | 2.3 | 2.3 | 2.3 | 2.3 | 2.3 |
| | Poly(meth)acrylate (E) | mass% | 10.3 | 10.3 | 10.3 | 10.3 | 10.3 | 10.3 | 10.3 | 10.3 |
| | Metal-based detergent (F) | mass% | 1.65 | 1.65 | 1.65 | 1.65 | 1.65 | 1.65 | 1.65 | 1.65 |
| | Zinc dithiophosphate (G) | mass% | 1.14 | 1.14 | 1.14 | 1.14 | 1.14 | 1.14 | 1.14 | 1.14 |
| | Other components | mass% | 6.16 | 6.16 | 6.16 | 6.16 | 6.16 | 6.16 | 6.16 | 6.16 |
| Properties of lubricating oil composition | Content of molybdenum derived from (B) | mass% of Mo | 0.070 | 0.070 | 0.070 | 0.070 | 0.030 | 0.070 | 0.070 | 0.070 |
| | Content [Z] of boron derived from (D) | mass% of B | 0.030 | 0.030 | 0.030 | 0.030 | 0.030 | 0.030 | 0.030 | 0.030 |
| | Content of metal derived from (F) | mass% of Metal | 0.200 | 0.200 | 0.200 | 0.200 | 0.200 | 0.200 | 0.200 | 0.200 |
| | [Y]/[X] | - | - | - | 0.10 | 0.20 | 0.20 | 0.50 | 1.00 | 0.25 |
| | [Z]/[X+Y] | - | 0.026 | 0.052 | 0.024 | 0.043 | 0.043 | 0.017 | 0.026 | 0.010 |
| | HTHS viscosity at 150°C | mPa·s | 2.6 | 2.6 | 2.6 | 2.6 | 2.6 | 2.6 | 2.6 | 2.6 |
| Evaluation | Friction coefficient | - | 0.054 | 0.057 | 0.054 | 0.051 | 0.051 | 0.043 | 0.058 | 0.065 |

From the results shown in Table 2, it can be confirmed that by using the ester-based ashless friction modifier (C1) in combination with the amine-based ashless friction modifier (C2), and allowing the mass ratio ([Y]/[X]) of the content [Y] of the amine-based ashless friction modifier (C2) to the content [X] of the ester-based ashless friction modifier (C1) to be less than 1.0, the friction-reducing effect can be more enhanced. In particular, it can be confirmed that the lubricating oil compositions of Examples 6 to 8, each having [Y]/[X] of more than 0.10 and less than 1.00, exhibit a highly excellent friction-reducing effect.

In addition, in Comparative Example 3, the ester-based ashless friction modifier (C1) is used in combination with the amine-based ashless friction modifier (C2), but the friction coefficient increases. The reason for this may be thought to be that in Comparative Example 3, the total amount of the ester-based ashless friction modifier (C1) and the amine-based ashless friction modifier (C2) is more than 1.8 mass% based on the total amount of the lubricating oil composition, so that the friction-reducing effect of the molybdenum compound (B) is inhibited.

**Table 3**

| | | | Example 6 | Example 10* |
|---|---|---|---|---|
| Composition | Lubricating base oil (A) | mass% | Balance | Balance |
| | Molybdenum compound (B) | mass% | 0.7 | 0.7 |
| | Ester-based friction modifier (C1) | mass% | 0.5 | 0.5 |
| | Amine-based friction modifier (C2) | mass% | 0.1 | 0.1 |
| | Borated succinimide (D) | mass% | 2.3 | - |
| | Poly(meth)acrylate (E) | mass% | 10.3 | 12.0 |
| | Metal-based detergent (F) | mass% | 1.65 | 1.65 |
| | Zinc dithiophosphate (G) | mass% | 1.14 | 1.14 |
| | Other components | mass% | 6.16 | 6.16 |
| Properties | Content of molybdenum derived from (B) | mass% of Mo | 0.070 | 0.070 |
| | Content of boron derived from (D) | mass% of B | 0.030 | - |
| | Content of metal derived from (F) | mass% of metal | 0.200 | 0.200 |
| | HTHS viscosity at 150°C | mPa·s | 2.6 | 2.6 |
| Evaluation | Friction coefficient | - | 0.051 | 0.059 |

From the results shown in Table 3, it can be confirmed that the lubricating oil composition of Example 6, including the molybdenum compound (B), the ester-based ashless friction modifier (C1) and/or the amine-based ashless friction modifier (C2), and the borated succinimide (D) exhibits a better friction-reducing effect, as compared with the lubricating oil composition of Example 10, including the molybdenum compound (B), the ester-based ashless friction modifier (C1) and/or the amine-based ashless friction modifier (C2), but not including the borated succinimide (D). The reason for this may be thought to be that in the lubricating oil composition of Example 6, by using the molybdenum compound (B), and the ester-based ashless friction modifier (C1) and/or the amine-based ashless friction modifier (C2), together with the borated succinimide (D), a friction-reducing effect based on the molybdenum compound (B) is more easily retained, and by the synergistic action with the molybdenum compound (B), and the ester-based ashless friction modifier (C1) and/or the amine-based ashless friction modifier (C2), the friction-reducing effect is more enhanced.

### Industrial Applicability

The lubricating oil composition of the present embodiment exhibits a good friction-reducing effect, and thus, the fuel consumption reducing properties can be enhanced. For this reason, the lubricating oil composition of the present embodiment can be suitably used for a variety of internal combustion engines of a four-wheel automobile, a two-wheel automobile, or the like. Further, among the internal combustion engines, the lubricating oil composition of the present embodiment can be particularly suitably used for a gasoline engine.

## Claims

1. A lubricating oil composition comprising:
a lubricating base oil (A);
a molybdenum compound (B);
an ashless friction modifier (C); and
a borated succinimide (D),
wherein the lubricating oil composition includes a binuclear organic molybdenum compound represented by the following general formula (I) as the molybdenum compound (B), with the content of the binuclear organic molybdenum compound as converted into molybdenum atoms being 0.030 mass% or more and 0.140 mass% or less based on the total amount of the lubricating oil composition; and
an ester-based ashless friction modifier (C1) and an amine-based ashless friction modifier (C2) as the ashless friction modifier (C), with the total content of the ester-based ashless friction modifier (C1) and the amine-based ashless friction modifier (C2) being more than 0.1 mass% and 1.8 mass% or less based on the total amount of the lubricating oil composition:
wherein R¹ to R⁴ each represents a hydrocarbon group having 4 to 22 carbon atoms, R¹ to R⁴ may be the same as or different from each other, and X¹ to X⁴ each represents a sulfur atom or an oxygen atom,
wherein the amine-based ashless friction modifier (C2) is an aliphatic amine-based compound having one or more hydroxyl groups in a molecule thereof,
wherein the mass ratio between the content of the amine-based ashless friction modifier (C2) and the content of the ester-based ashless friction modifier (C1) [the content of the amine-based ashless friction modifier (C2)/the content of the ester-based ashless friction modifier (C1)] is 0.15 or more and 0.80 or less.

2. The lubricating oil composition according to claim 1, wherein the ester-based ashless friction modifier (C1) is an ester compound having one or more hydroxyl groups in a molecule thereof.

3. The lubricating oil composition according to claim 2, wherein the ester compound having one or more hydroxyl groups in a molecule thereof is glycerin monooleate.

4. The lubricating oil composition according to any one of claims 1 to 3, wherein a total content of the ester-based ashless friction modifier (C1) and the amine-based ashless friction modifier (C2) based on the total amount of the ashless friction modifier (C) is 80 mass% or more, preferably 90 mass% or more, and more preferably 100 mass%.

5. The lubricating oil composition according to any one of claims 1 to 4, wherein the content of the borated succinimide (D) as converted into boron atoms is 0.050 mass% or less based on the total amount of the lubricating oil composition.

6. The lubricating oil composition according to any one of claims 1 to 5, wherein the mass ratio of the content of the borated succinimide (D) as converted into boron atoms to the total content of the ester-based ashless friction modifier (C1) and the amine-based ashless friction modifier (C2) [the content of the borated succinimide (D) as converted into boron atoms/(the content of the ester-based ashless friction modifier (C1) + the content of the amine-based ashless friction modifier (C2))] is 0.011 or more.

7. The lubricating oil composition according to any one of claims 1 to 6, further comprising a poly(meth)acrylate (E).

8. The lubricating oil composition according to any one of claims 1 to 7, further comprising a metal-based detergent (F).

9. The lubricating oil composition according to any one of claims 1 to 8, further comprising zinc dithiophosphate (G).

10. The lubricating oil composition according to any one of claims 1 to 9, wherein the lubricating base oil (A) is one or more selected from mineral oils or synthetic oils classified into Group 3 and Group 4 in the base oil classification of the American Petroleum Institute.

11. The lubricating oil composition according to any one of claims 1 to 10, which is used for an internal combustion engine.

12. A method for reducing friction of an internal combustion engine, comprising adding the lubricating oil composition according to any one of claims 1 to 10 to an internal combustion engine.

## Patentansprüche

1. Schmiermittelzusammensetzung, umfassend:
ein Schmiermittelbasisöl (A);
eine Molybdänverbindung (B);
einen aschefreien Reibungsmodifizierer (C); und
ein boriertes Succinimid (D),
worin die Schmiermittelzusammensetzung eine zweikernige organische Molybdänverbindung als Molybdänverbindung (B) enthält, die durch die folgende allgemeine Formel (I) dargestellt wird, wobei der Gehalt der zweikernigen organischen Molybdänverbindung, umgerechnet in Molybdänatome, 0,030 Massen-% oder mehr und 0,140 Massen-% oder weniger, bezogen auf die Gesamtmenge der Schmiermittelzusammensetzung, beträgt; und
einen esterbasierten aschefreien Reibungsmodifizierer (C1) und einen aminbasierten aschefreien Reibungsmodifizierer (C2) als den aschefreien Reibungsmodifizierer (C), wobei der Gesamtgehalt des esterbasierten aschefreien Reibungsmodifizierers (C1) und des aminbasierten aschefreien Reibungsmodifizierers (C2) mehr als 0,1 Massen-% und 1,8 Massen-% oder weniger, bezogen auf die Gesamtmenge der Schmierölzusammensetzung, beträgt:
worin R¹ bis R⁴ jeweils eine Kohlenwasserstoffgruppe mit 4 bis 22 Kohlenstoffatomen darstellen, R¹ bis R⁴ die gleichen oder voneinander verschiedene sein können und X¹ bis X⁴ jeweils ein Schwefelatom oder ein Sauerstoffatom darstellen,
worin der aminbasierte aschefreie Reibungsmodifizierer (C2) eine aliphatische aminbasierte Verbindung mit einer oder mehreren Hydroxylgruppen in einem Molekül davon ist,
worin das Massenverhältnis zwischen dem Gehalt des aminbasierten aschefreien Reibungsmodifizierers (C2) und dem Gehalt des esterbasierten aschefreien Reibungsmodifizierers (C1) [Gehalt des aminbasierten aschefreien Reibungsmodifizierers (C2)/Gehalt des esterbasierten aschefreien Reibungsmodifizierers (C1)] 0,15 oder mehr und 0,80 oder weniger beträgt.

2. Schmierölzusammensetzung gemäß Anspruch 1, worin der esterbasierte aschefreie Reibungsmodifizierer (C1) eine Esterverbindung mit einer oder mehreren Hydroxylgruppen in einem Molekül davon ist.

3. Schmierölzusammensetzung gemäß Anspruch 2, worin die Esterverbindung mit einer oder mehreren Hydroxylgruppen in einem Molekül davon Glycerinmonooleat ist.

4. Schmierölzusammensetzung gemäß einem der Ansprüche 1 bis 3, worin ein Gesamtgehalt des esterbasierten aschefreien Reibungsmodifizierers (C1) und des aminbasierten aschefreien Reibungsmodifizierers (C2), bezogen auf die Gesamtmenge des aschefreien Reibungsmodifizierers (C), 80 Massen-% oder mehr, bevorzugt 90 Massen-% oder mehr, und bevorzugter 100 Massen-% beträgt.

5. Schmierölzusammensetzung gemäß einem der Ansprüche 1 bis 4, worin der Gehalt des borierten Succinimids (D), umgerechnet in Boratome, 0,050 Massen-% oder weniger, bezogen auf die Gesamtmenge der Schmierölzusammensetzung, beträgt.

6. Schmierölzusammensetzung gemäß einem der Ansprüche 1 bis 5, worin das Massenverhältnis des Gehalts des borierten Succinimids (D), umgerechnet in Boratome, zum Gesamtgehalt des esterbasierten aschefreien Reibungsmodifizierers (C1) und des aminbasierten aschefreien Reibungsmodifizierers (C2) [Gehalt des borierten Succinimids (D), umgerechnet in Boratome/(Gehalt des esterbasierten aschefreien Reibungsmodifizierers (C1) + Gehalt des aminbasierten aschefreien Reibungsmodifizierers (C2))] 0,11 oder mehr ist.

7. Schmierölzusammensetzung gemäß einem der Ansprüche 1 bis 6, ferner umfassend ein Poly(meth)acrylat (E).

8. Schmierölzusammensetzung gemäß einem der Ansprüche 1 bis 7, ferner umfassend ein metallbasiertes Detergenz (F).

9. Schmierölzusammensetzung gemäß einem der Ansprüche 1 bis 8, ferner umfassend Zinkdithiophosphat (G).

10. Schmierölzusammensetzung gemäß einem der Ansprüche 1 bis 9, worin das Schmiermittelbasisöl (A) eines oder mehrere ist, ausgewählt aus Mineralölen oder synthetischen Ölen, die in der Basisölklassifikation des American Petroleum Institute in Gruppe 3 und Gruppe 4 eingestuft sind.

11. Schmierölzusammensetzung gemäß einem der Ansprüche 1 bis 10, die für einen Verbrennungsmotor verwendet wird.

12. Verfahren zur Verringerung der Reibung eines Verbrennungsmotors, umfassend die Zugabe der Schmiermittelzusammensetzung gemäß einem der Ansprüche 1 bis 10 zu einem Verbrennungsmotor.

## Revendications

1. Composition d'huile lubrifiante comprenant :
une huile de base lubrifiante (A) ;
un composé de molybdène (B) ;
un modificateur (C) de frottement sans cendres ; et
un succinimide boraté (D),
dans laquelle la composition d'huile lubrifiante inclut un composé de molybdène organique binucléaire représenté par la formule générale (I) suivante en tant que composé de molybdène (B), avec la teneur en composé de molybdène organique binucléaire tel que converti en atomes de molybdène étant de 0,030 % en masse ou plus et de 0,140 % en masse ou moins sur la base de la quantité totale de la composition d'huile lubrifiante ; et
un modificateur (C1) de frottement sans cendres à base d'ester et un modificateur (C2) de frottement sans cendres à base d'amine en tant que modificateur (C) de frottement sans cendres, avec la teneur totale en modificateur (C1) de frottement sans cendres à base d'ester et en modificateur (C2) de frottement sans cendres à base d'amine étant supérieure à 0,1 % en masse et de 1,8 % en masse ou moins sur la base de la quantité totale de la composition d'huile lubrifiante :
dans laquelle R¹ à R⁴ représentent chacun un groupe hydrocarbure présentant 4 à 22 atomes de carbone, R¹ à R⁴ peuvent être identiques les uns aux autres ou différents les uns des autres, et X¹ à X⁴ représentent chacun un atome de soufre ou un atome d'oxygène,
dans laquelle le modificateur (C2) de frottement sans cendres à base d'amine est un composé à base d'amine aliphatique présentant un ou plusieurs groupes hydroxyles dans une molécule de celui-ci,
dans laquelle le rapport en masse entre la teneur en modificateur (C2) de frottement sans cendres à base d'amine et la teneur en modificateur (C1) de frottement sans cendres à base d'ester [la teneur en modificateur (C2) de frottement sans cendres à base d'amine/la teneur en modificateur (C1) de frottement sans cendres à base d'ester] est de 0,15 ou plus et de 0,80 ou moins.

2. Composition d'huile lubrifiante selon la revendication 1, dans laquelle le modificateur (C1) de frottement sans cendres à base d'ester est un composé ester présentant un ou plusieurs groupes hydroxyles dans une molécule de celui-ci.

3. Composition d'huile lubrifiante selon la revendication 2, dans laquelle le composé ester présentant un ou plusieurs groupes hydroxyles dans une molécule de celui-ci est du monooléate de glycérine.

4. Composition d'huile lubrifiante selon l'une quelconque des revendications 1 à 3, dans laquelle une teneur totale en modificateur (C1) de frottement sans cendres à base d'ester et en modificateur (C2) de frottement sans cendres à base d'amine sur la base de la quantité totale du modificateur (C) de frottement sans cendres est de 80 % en masse ou plus, préférentiellement de 90 % en masse ou plus, et plus préférentiellement de 100 % en masse.

5. Composition d'huile lubrifiante selon l'une quelconque des revendications 1 à 4, dans laquelle la teneur en succinimide boraté (D) tel que converti en atomes de bore est de 0,050 % en masse ou moins sur la base de la quantité totale de la composition d'huile lubrifiante.

6. Composition d'huile lubrifiante selon l'une quelconque des revendications 1 à 5, dans laquelle le rapport en masse de la teneur en succinimide boraté (D) tel que converti en atomes de bore à la teneur totale en modificateur (C1) de frottement sans cendres à base d'ester et en modificateur (C2) de frottement sans cendres à base d'amine [la teneur en succinimide boraté (D) tel que converti en atomes de bore/(la teneur en modificateur (C1) de frottement sans cendres à base d'ester + la teneur en modificateur (C2) de frottement sans cendres à base d'amine)] est de 0,011 ou plus.

7. Composition d'huile lubrifiante selon l'une quelconque des revendications 1 à 6, comprenant en outre un poly(méth)acrylate (E).

8. Composition d'huile lubrifiante selon l'une quelconque des revendications 1 à 7, comprenant en outre un détergent (F) à base de métal.

9. Composition d'huile lubrifiante selon l'une quelconque des revendications 1 à 8, comprenant en outre du dithiophosphate de zinc (G).

10. Composition d'huile lubrifiante selon l'une quelconque des revendications 1 à 9, dans laquelle l'huile de base lubrifiante (A) est une ou plusieurs choisies parmi les huiles minérales ou les huiles synthétiques classées dans le Groupe 3 et le Groupe 4 dans la classification des huiles de base de l'American Petroleum Institute.

11. Composition d'huile lubrifiante selon l'une quelconque des revendications 1 à 10, qui est utilisée pour un moteur à combustion interne.

12. Procédé de réduction du frottement d'un moteur à combustion interne, comprenant l'ajout de la composition d'huile lubrifiante selon l'une quelconque des revendications 1 à 10 à un moteur à combustion interne.
